

Patented Mar. 30, 1954

2,673,801

# UNITED STATES PATENT OFFICE

2,673,801

## PRODUCTION OF COLOR PHOTOGRAPHIC IMAGES

Jacob Joseph Jennen, Antwerp, Belgium, assignor to Gevaert Photo-Producten N. V., Mortsel, Belgium, a Belgian company

No Drawing. Application November 22, 1949,  
Serial No. 128,913

Claims priority, application Great Britain  
November 23, 1948

8 Claims. (Cl. 95—6)

1

This invention relates to a process for the production of color photographic images by color development in the presence of a color coupler, to photographic developers, photographic material containing such couplers, and photographic images obtained by such a process.

It is known that a colored image may be formed by developing a reducible silver salt image in the presence of a compound which during the development couples with the oxidation product of the developing agent and forms a dyestuff which is deposited on the developed silver grains.

To develop magenta dyestuff images, compounds have hitherto been used which contain an active methylene group such as pyrazolones and cyanacetic acid derivatives.

I have now found that a magenta image may also be obtained when a compound is used as a color coupler which does not contain such an active methylene group.

It is an object of my present invention to provide a new process for the production of color photographic images by color development.

A further object of this invention is to provide new photographic developers containing a color coupler.

Another object of the invention is to provide new photographic material containing a color coupler.

Further objects will appear from the following description.

According to my invention, a reducible silver salt image is developed with a primary aromatic amino developing agent in the presence of a compound corresponding to the following Formula I:

I



or to a tautomeric form thereof, corresponding, for instance, to Formula II or III

II



III



In all these Formulae I, II and III, Z represents the nonmetallic atoms required for completing an aromatic nucleus, it being understood that the

aromatic nucleus may be isocyclic, heterocyclic or polycyclic. The polycyclic nucleus completed by Z may contain at least one further

—NH—NH—CO—

5 group so as to have a double indazolone compound. The compound, as completed by Z, may also contain two or more nuclei linked by a chemical bound or by a bi- or poly-valent atom or group, such as



Bearing in mind that the new color coupler may be represented by Formula II, it is believed that coupling with the oxidation products of the developing agent occurs at the N-atom in ortho-position to the OH group. This assumption is supported by the coupling reaction of a diazo compound with para-cresol and beta-naphthol which also occurs in ortho-position to the OH group, and with 3,4-dimethyl-5-hydroxy pyrazole which probably occurs in the same manner. The dyestuff formed from the new couplers may be written as follows



These formulae are analogous to the formula LV of Baker for 2-substituted indazolone (J. Chem. Soc., London (1945) 267).

By this process, dyestuff images may be obtained which have an absorption maximum at about 530-530 m $\mu$ .

Color couplers according to Formula I may be obtained by causing a molecule of water to split off from aromatic, dihydro-aromatic or heterocyclic mono- or poly-(ortho-hydrazino carboxylic acids) according to the method described by K. Pfannsteil and J. Janecke in "Berichte" 75 (1942) 1101.

Sometimes, the preparation of one of said hydrazino acids yields directly the corresponding indazolone because the hydrazino acid although occurring at an intermediate stage cannot be isolated.

The color coupler according to my present invention may also be obtained in a manner anal-

ogous to the preparation of indazolone-4-carboxylic acid of 5- or 6-chloro-indazolone.

The preparation of indazolone-4-carboxylic acid may be effected by diazotizing 3,4-benzoisoxazolone-4-carboxylic acid and reducing the resulting diazo compound with  $\text{SO}_2$  (J. pr. Chem. [2] 146 (1936) 134).

5- or 6-chloro indazolone may be prepared by treating 2-carboxy-4- or 5-chloro phenyl hydrazone of ethyl glyoxylate with concentrated sulphuric acid (J. Org. Chem. 12 (1947) 53).

3,4-pyrazolono-pyrazolone may be prepared by condensing hydrazine and 4-isonitroso-pyrazolone-3-carboxylic acid (J. pr. Chem. [2] 51 (1895) 63). This 3,4-pyrazolono-pyrazolone may be written in many tautomeric forms, one of which is represented by the following Formula XX:

XX



Most of these color couplers are converted into a yellow product when in an oxidizing medium such as a bath for removal of the silver so that a yellow reversal image, which results from the oxidation of the residual color coupler in the bath for removing the silver, is added to the dyestuff image formed on color development. If this is undesirable, the formation of the yellow product may be avoided by treating the color developed emulsion layer, before removing the silver, with a bath containing formaldehyde, a formaldehyde-yielding compound, or another aldehyde. Such an aldehyde is supposed to react with the  $-\text{NH}-\text{NH}-\text{CO}-$  group of the coupler, avoiding in this way any subsequent coupling or formation of yellow oxidation products.

The dyestuffs obtained on color development with the color couplers according to the present invention are more stable to acid than those obtained with the known pyrazolones, and those which contain a substituent rendering them fast to diffusion are not removable from the emulsion layer by washing.

The said new color couplers may further be used in the developing solution or in a colloid layer, in the latter case either in a light-sensitive layer or in a non-light-sensitive layer adjacent to a sensitive layer or separated therefrom by a water-permeable colloid layer.

The aromatic amino compounds which may be used as developing agents in accordance with the present invention include the mono-, di- and tri-amino aryl compounds. Among the mono-amino developing agents may be mentioned amino phenols and amino cresols and their halogen derivatives, and amino naphthols.

The developing agents which are preferred and gave the best results when used according to my invention are the aromatic ortho and paradiamines, such as para-phenylene diamine and its substitution products.

The following examples are given to illustrate the invention, without limiting, however, the scope thereof.

#### Example 1

1.1 g. indazolone according to Formula IV:

IV



and prepared, for instance, according to K. Pfannstiel and J. Janecke, "Berichte" 75 (1942) 1104, are dissolved in 20 cc. of an aqueous solution of sodium carbonate 10% and added to 100 cc. of a photographic silver halide emulsion prepared from 2.75 g.  $\text{AgNO}_3$ . This emulsion is coated onto a support, exposed and developed in a solution obtained by mixing equal parts of the following solutions:

|                                                   |    |     |
|---------------------------------------------------|----|-----|
| (A) N,N-diethyl-p-phenylene diamine hydrochloride | g  | 6   |
| Water to                                          | cc | 500 |
| (B) Potassium carbonate                           | g  | 75  |
| Potassium bromide                                 | g  | 2.5 |
| Water to                                          | cc | 500 |

A magenta dyestuff image with an absorption maximum at  $550 \text{ m}\mu$  is formed.

#### Example 2

1 g. 4-chloro-indazolone according to Formula V:

V



which has been prepared according to "Berichte" 75 (1942) 1106 is dissolved in 22 cc. of an aqueous solution of sodium carbonate 5% and added to 100 cc. of a positive photographic silver halide emulsion. This emulsion is coated onto a support, exposed and developed in a solution obtained by mixing equal parts of the following solutions:

|                                              |    |     |
|----------------------------------------------|----|-----|
| (A) N,N-diethyl-p-phenylene diamine sulphate | g  | 3.2 |
| Water to                                     | cc | 500 |
| (B) Potassium carbonate                      | g  | 75  |
| Potassium bromide                            | g  | 2.5 |

Water to

A magenta dyestuff image is formed.

#### Example 3

11 g. 3,5-dichloro-2-amino benzoic acid are dissolved in 50 cc. of a concentrated aqueous solution of hydrochloric acid and 350 cc. water. To this solution are added 100 cc. of an aqueous solution of sodium nitrite 5%. Next, the mixture is added during 10 minutes to 750 cc. of an aqueous saturated solution of  $\text{SO}_2$  while  $\text{SO}_2$  gas is continuously conducted into said solution. After complete addition,  $\text{SO}_2$  is continued to be introduced for another 30 minutes, whereupon the mixture is boiled during 30 minutes, cooled and filtered with suction. The product obtained is recrystallized with ethanol. Melting point 227-228° C. N content calculated 13.79, found 13.50. It is believed to be 5,7-dichloro-indazolone corresponding to Formula VI:

VI



2 g. of the indazolone derivative prepared as indicated above are dissolved in 50 cc. water and 10 cc. of an aqueous solution of sodium hydroxide.

2 N and added to 1 litre of a mixture of equal parts of the following solutions:

|                                              |    |     |    |
|----------------------------------------------|----|-----|----|
| (A) N,N-diethyl-p-phenylene diamine sulphate | g  | 3.2 | 5  |
| Sodium sulfite                               | g  | 5   |    |
| Water to                                     | cc | 500 |    |
| (B) Potassium carbonate                      | g  | 75  | 10 |
| Potassium bromide                            | g  | 2.5 |    |
| Water to                                     | cc | 500 |    |

An exposed positive motion picture film is developed in the developer thus prepared and a magenta image with absorption maxima at 542 and 581 m $\mu$  is formed.

*Example 4*

6 g. 4-nitro-indazolone according to Formula VII:

VII



prepared according to "Berichte" 75 (1942) 1105 are dissolved in 100 cc. acetone and 20 cc. of an aqueous solution of sodium hydroxide 2 N and added to 1 litre of a mixture of equal parts of the following solutions:

|                                              |    |     |    |
|----------------------------------------------|----|-----|----|
| (A) N,N-diethyl-p-phenylene diamine sulphate | g  | 3.2 | 25 |
| Water to                                     | cc | 500 |    |
| (B) Potassium carbonate                      | g  | 75  |    |
| Potassium bromide                            | g  | 2.5 |    |
| Potassium metal bisulfite                    | g  | 1   |    |
| Water to                                     | cc | 500 |    |

In the developing solution thus prepared, an exposed positive motion picture film is developed and a magenta image with an absorption maximum of 575 m $\mu$  is obtained.

*Example 5*

8.5 g. 4-sulfo-1-amino benzol-2-carboxylic acid are dispersed in 32 cc. of a concentrated aqueous solution of hydrochloric acid. Successively, 64 cc. of an aqueous solution of sodium nitrite 5% are added to the suspension, and then 225 cc. water. The whole is brought slowly into 480 cc. of a solution of SO<sub>2</sub> while SO<sub>2</sub> gas is continuously conducted into that solution. After complete addition, SO<sub>2</sub> is introduced for yet half an hour. Next, the volume of the mixture is reduced to about 150 cc. by evaporation. The mixture is cooled and filtered with suction. The product separated is recrystallized in a little amount of water. It melts above 300° C. and is believed to be indazolone-5-sulfonic acid corresponding to Formula VIII:

VIII



N content calculated 13.08, found 13.51. S content calculated 14.95, found 15.03.

2 g. of this indazolone-5-sulfonic acid are added to a mixture of equal parts of the following solution:

|                                              |    |     |    |
|----------------------------------------------|----|-----|----|
| (A) N,N-diethyl-p-phenylene diamine sulphate | g  | 3.2 | 70 |
| Water to                                     | cc | 500 |    |
| (B) Potassium carbonate                      | g  | 75  |    |
| Potassium bromide                            | g  | 2.5 |    |
| Water to                                     | cc | 500 | 75 |

An exposed positive motion picture film is developed in the color developer thus prepared and a bluish magenta image is formed.

*Example 6*

6.6 g. 6-amino-indazolone-hydrochloride, prepared according to "Berichte" 75 (1912) 1107, and 5.1 g. 2-chlorobenzothiazole are dissolved in 100 cc. absolute ethanol. The solution is evaporated on the water bath. The residue is washed by boiling with ether and then with water. The washed residue is dissolved in 200 cc. ethanol. The volume of the solution is reduced to 20 cc. The product which precipitates after cooling is filtered with suction. It melts at 252-255° C. After washing by boiling with water and then with acetone, the melting point may be raised to 270-272° C.

S content calculated 11.34, found 12.73.

20 The product is believed to be 6(2'-benzothiazolyl amino)indazolone according to Formula IX:

IX



25 2 g. of this indazolone derivative are dissolved in 20 cc. of a methanolic solution of potassium hydroxide N and added to 1 litre of a mixture of equal parts of the following solutions:

|                                              |    |     |    |
|----------------------------------------------|----|-----|----|
| (A) N,N-diethyl-p-phenylene diamine sulphate | g  | 3.2 | 35 |
| Sodiumsulfite                                | g  | 5   |    |
| Water to                                     | cc | 500 |    |
| (B) Potassium carbonate                      | g  | 75  |    |
| Potassium bromide                            | g  | 2.5 |    |
| Water to                                     | cc | 500 |    |

40 An exposed positive motion picture film is developed in the developer thus prepared and a bluish magenta image is formed. Absorption maximum 576 m $\mu$ .

*Example 7*

45 A solution of 2.2 g. 6-amino-indazolone hydrochloride and 3 g. 2-methyl-mercapto benzothiazole dimethylsulphate in 20 cc. pyridine is refluxed for 30 minutes and then poured into water. The precipitate is filtered with suction and recrystallized from ethanol. Melting point is 262-264° C. The product is believed to be 6(1'-methyl - benzothiazolylidene-2')aminoindazolone according to Formula X:

X



60 N content calculated 18.85, found 18.16. S content calculated 10.77, found 11.26.

65 0.2 g. of this indazolone derivative is dissolved in 50 cc. alcoholic solution of potassium hydroxide N and added to 100 cc. of a mixture of equal parts of the following solutions:

|                                              |    |     |    |
|----------------------------------------------|----|-----|----|
| (A) N,N-diethyl-p-phenylene diamine sulphate | g  | 3.2 | 70 |
| Sodium sulfite                               | g  | 5   |    |
| Water to                                     | cc | 500 |    |
| (B) Potassium carbonate                      | g  | 75  |    |
| Potassium bromide                            | g  | 2.5 |    |
| Water to                                     | cc | 500 | 75 |

By developing an exposed positive motion picture film in the developer thus prepared, a magenta image with an absorption maximum at 567 m $\mu$  is formed.

Example 8

A mixture of 5.5 g. 6-amino-indazolone-hydrochloride, 3.7 g. phthalic acid anhydride and 5 cc. pyridine is heated for 30 minutes at 180° C. on an oil bath. The mixture is cooled and the solid mass obtained is washed by boiling with water and next with acetone. Melting point is 304-305° C. N content calculated 15.05, found 14.79. The product is believed to be 6-phthal-imido indazolone corresponding to Formula XI:

XI



0.2 g. of this indazolone derivative is dissolved in 50 cc. alcoholic solution of potassium hydroxide N and added to 100 cc. of a mixture of equal parts of the following solutions:

|                                 |                   |      |     |
|---------------------------------|-------------------|------|-----|
| (A) N,N-diethyl-p-phenylene di- | amine sulfate     | g..  | 3.2 |
|                                 | Sodium sulfite    | g..  | 5   |
|                                 | Water to          | cc.. | 500 |
| (B) Potassium carbonate         | g..               | 75   | 25  |
|                                 | Potassium bromide | g..  | 2.5 |
|                                 | Water to          | cc.. | 500 |

By developing an exposed positive motion picture film in the developer thus prepared, a magenta image is formed.

Example 9

A solution of 5 g. 7-amino-indazolone hydrochloride, prepared according to "Berichte" 75 (1942) 1107, and 9 g. octadecenyl succinic acid anhydride in 35 cc. pyridine is refluxed for two hours and poured into 350 cc. water to which 35 cc. of a concentrated aqueous solution of hydrochloric acid are added. The precipitate obtained is separated by filtration with suction. The residue is washed by boiling with a little acetone, then with methanol and finally recrystallized with glycol acetate. Melting point is 190-191° C. This product corresponds to the probable Formula XII:

XII



N content calculated 8.41, found 8.32 and 8.40. 1 g. of this 7-octadecenyl - succinyl - amino-indazolone dissolved in 2.5 cc. ethanol and 2.5 cc. of an aqueous solution of sodium hydroxide 2 N is added to 100 cc. of an emulsion for positive motion picture film. This emulsion is coated onto a support, exposed and developed in a solution obtained by mixing equal parts of the following solutions:

|                                 |                   |      |     |
|---------------------------------|-------------------|------|-----|
| (A) N,N-diethyl-p-phenylene di- | amine sulfate     | g..  | 3.2 |
|                                 | Sodium sulfite    | g..  | 5   |
|                                 | Water to          | cc.. | 500 |
| (B) Potassium carbonate         | g..               | 75   | 60  |
|                                 | Potassium bromide | g..  | 2.5 |
|                                 | Water to          | cc.. | 500 |

75

A magenta image with an absorption maximum at 530 m $\mu$  is obtained. This coupler does not diffuse.

A magenta image with an absorption maximum at 562 m $\mu$  is obtained. This coupler does not diffuse. The 4, 5 and 6 - octadecenyl - succinyl-amino-indazolones may be prepared and used in the same way.

Example 10

A solution of 1.1 g. 6-amino-indazolone-hydrochloride and 1.1 g. of the copolymer of styrene and maleic acid anhydride in 5.5 cc. pyridine is boiled for 5 hours. The reaction mixture is washed with boiling water, and then with boiling methanol. A product melting above 300° C. and corresponding to Formula XIII:



wherein x is a positive integer, is obtained.

N content calculated 11.96, found 11.03%.

1 g. of this product is dissolved in 30 cc. of a concentrated aqueous solution of NH<sub>3</sub> by heating on the water bath and added to 100 cc. of an emulsion for a positive motion picture film. This emulsion is coated onto a support, exposed and developed in a solution obtained by mixing equal parts of the following solutions:

|                                 |                   |      |     |
|---------------------------------|-------------------|------|-----|
| (A) N,N-diethyl-p-phenylene-di- | amine sulfate     | g..  | 3.2 |
|                                 | Sodium sulfite    | g..  | 5   |
|                                 | Water to          | cc.. | 500 |
| (B) Potassium carbonate         | g..               | 75   | 30  |
|                                 | Potassium bromide | g..  | 2.5 |
|                                 | Water to          | cc.. | 500 |

A magenta image is obtained. This coupler does not diffuse.

Example 11

3.2 g. 5-amino-indazolone - hydrochloride prepared according to "Berichte" 75 (1942) 1107, 6 g. stearic acid chloride and 45 cc. pyridine are refluxed for 5 hours. The residue is washed by boiling first with water, then with acetone and finally with methanol. 5 - stearoyl-amino - indazolone melting at 218-220° C. and corresponding to Formula XIV:



55 is obtained.

N content calculated 10.12, found 10.03 and 10.20.

1 g. of this product is dissolved in 3 cc. of an ethanolic solution of potassium hydroxide N and 7 cc. methanol and added to 100 cc. of an emulsion for positive motion picture film. This emulsion is coated onto a support, exposed and developed in a solution obtained by mixing equal parts of the following solutions:

|                                 |                   |      |     |
|---------------------------------|-------------------|------|-----|
| (A) N,N-diethyl-p-phenylene di- | amine sulfate     | g..  | 3.2 |
|                                 | Sodium sulfite    | g..  | 5   |
|                                 | Water to          | cc.. | 500 |
| (B) Potassium carbonate         | g..               | 75   | 60  |
|                                 | Potassium bromide | g..  | 2.5 |
|                                 | Water to          | cc.. | 500 |

A magenta image with an absorption maximum at 530 m $\mu$  is obtained. This coupler does not diffuse.

## Example 12

0.2 g. of the bis-indazolone derivative called hereinafter 5-(indazolonyl-5')-indazolone, corresponding to Formula XV:

XV



and prepared according to Gazz. Chim. Ital. 66 (1936) 17, are dissolved in 5 cc. ethanolic solution of potassium hydroxide N and added to a solution obtained by mixing 50 cc. of each of the following solutions:

|                                                    |    |     |
|----------------------------------------------------|----|-----|
| (A) N,N - diethyl - p - phenylene diamine sulphate | g  | 3.2 |
| Sodium sulfite                                     | g  | 5   |
| Water to                                           | cc | 500 |
| (B) Potassium carbonate                            | g  | 75  |
| Potassium bromide                                  | g  | 2.5 |
| Water to                                           | cc | 500 |

By developing an exposed positive motion picture film in the developer thus prepared, a bluish magenta image with an absorption maximum at 580  $\mu$  is obtained.

## Example 13

0.2 g. 2,6-dimethyl-4-hydrazino nicotinic anhydride corresponding to Formula XVI:

XVI



and prepared according to "Berichte" 36 (1903) 519 are dissolved in 5 cc. of an aqueous solution of potassium hydroxide N/10 and added to a solution obtained by mixing 50 cc. of each of the following solutions:

|                                                    |    |     |
|----------------------------------------------------|----|-----|
| (A) N,N - diethyl - p - phenylene diamine sulphate | g  | 3.2 |
| Water to                                           | cc | 500 |
| (B) Potassium carbonate                            | g  | 75  |
| Potassium bromide                                  | g  | 2.5 |

Water to

By developing an exposed positive motion picture film in the developer thus prepared, a bluish magenta image with an absorption maximum at 579  $\mu$  is obtained.

## Example 14

6.7-imidazo-indazolone is prepared by the same method as 6.7-imidazo-indazole, the preparation of which is described in Jl. Am. Chem. Soc., 48 (1926) 1104. It suffices to replace the starting material 6-amino-indazole by 6-amino-indazolone. After recrystallization in glacial acetic acid, the product melts above 300° C. and corresponds to Formula XVII:

XVII



1 g. of this product is dissolved in 20 cc. of an aqueous solution of potassium hydroxide N/2 and added to 100 cc. of an emulsion for positive motion picture film. This emulsion is coated onto a support, exposed and developed in a solution ob-

tained by mixing equal parts of the following solutions:

|                                                    |    |     |
|----------------------------------------------------|----|-----|
| (A) N,N - diethyl - p - phenylene diamine sulphate | g  | 3.2 |
| Water to                                           | cc | 500 |
| (B) Potassium carbonate                            | g  | 75  |
| Potassium bromide                                  | g  | 2.5 |
| Water to                                           | cc | 500 |

10 A violet image is obtained.

## Example 15

1 g. of the bis-indazolone described as hexahydrobenzodipyrizolone corresponding to Formula XVIII:

XVIII



and prepared according to Jl. für pr. Chemie, [2] 51 (1895) 66, are dissolved in 22 cc. of an aqueous solution of NaOH 2 N and 5 cc. ethyl alcohol by heating and added to 100 cc. of an emulsion for positive motion picture film. This emulsion is coated onto a support, exposed and developed in a solution obtained by mixing equal parts of the following solutions:

|                                                    |    |     |
|----------------------------------------------------|----|-----|
| (A) N,N - diethyl - p - phenylene diamine sulphate | g  | 3.2 |
| Water to                                           | cc | 500 |
| (B) Potassium carbonate                            | g  | 75  |
| Potassium bromide                                  | g  | 2.5 |
| Water to                                           | cc | 500 |

20 A bluish image is formed.

## Example 16

To 14 g. diamino diphenyl methane dicarboxylic acid and 40 cc. concentrated aqueous solution of hydrochloric acid, 35 cc. of an aqueous solution of sodium nitrite 10% are added while cooling with ice.

The reaction mixture is filtered. The filtrate is added in 30 minutes drop by drop to 400 cc. of a saturated aqueous solution of sulphurous anhydride while cooling with ice-water and conducting  $SO_2$  into the reaction mixture. After complete addition, introduction of  $SO_2$  is continued for another 30 minutes. 400 cc. 25 water are then added and the whole is boiled for one hour, whereupon the mixture is filtered and the filtrate cooled. The precipitate is recrystallized from ethyl alcohol. The 5-methylene-bis-indazolone obtained corresponds to Formula 50 XIX:

XIX



55 Melting point is above 310° C.

2 g. of this product are dissolved in 40 cc. of an aqueous solution of sodium carbonate 10% and added to 1 litre of a mixture of equal parts of the 60 following solutions:

|                                                         |    |     |
|---------------------------------------------------------|----|-----|
| (A) N,N - diethyl - p - phenylene diamine hydrochloride | g  | 6   |
| Sodium sulfite                                          | g  | 5   |
| Water to                                                | cc | 500 |
| (B) Potassium carbonate                                 | g  | 75  |
| Potassium bromide                                       | g  | 2.5 |
| Water to                                                | cc | 500 |

70 A magenta dyestuff image with an absorption maximum at 530  $\mu$  is formed.

I claim:

1. Process for the production of a colored photographic image, which comprises developing a reducible silver salt image in a photographic element by means of a primary aromatic amino developing agent in the presence of a color coupler having a formula selected from the group consisting of Formula I:

I



and tautomeric forms of Formula I, wherein Z represents the non-metallic atoms required for completing an aromatic nucleus. 15

2. Photographic developer containing a primary aromatic amino developing agent and a color coupler having a formula selected from the group consisting of Formula I:

I



and tautomeric forms of Formula I, wherein Z represents the non-metallic atoms required for completing an aromatic nucleus.

3. A photographic developer containing a primary aromatic amino developing agent and 5-(indazolonyl-5')-indazolone.

4. A photographic developer containing a primary aromatic amino developing agent and 5-methylene-bis-indazolone.

5. A photographic material comprising a silver halide emulsion layer and a colloid layer, containing an octadecenyl-succinyl-amino-indazolone.

6. A photographic material comprising a silver 40

halide emulsion layer and a colloid layer, containing a condensation product of 6-amino-indazolone and a copolymer of styrene and maleic acid anhydride.

5 7. A photographic material comprising a silver halide emulsion layer and a colloid layer, containing 5-stearoyl-amino-indazolone.

8. A photographic material comprising a silver halide emulsion layer and a colloid layer, containing a color coupler having a formula selected from the group consisting of Formula I:



and tautomeric forms of Formula I, wherein Z represents the non-metallic atoms required for completing an aromatic nucleus.

JACOB JOSEPH JENNEN.

References Cited in the file of this patent  
UNITED STATES PATENTS

| 25 | Number    | Name       | Date           |
|----|-----------|------------|----------------|
|    | 742,405   | Eichengrun | Oct. 27, 1903  |
|    | 2,200,306 | Schneider  | May 14, 1940   |
|    | 2,213,986 | Kendall    | Sept. 10, 1940 |
|    | 2,353,754 | Peterson   | July 18, 1944  |

FOREIGN PATENTS

| Number  | Country       | Date         |
|---------|---------------|--------------|
| 524,557 | Great Britain | Aug. 8, 1940 |
| 577,804 | Great Britain | May 31, 1946 |

OTHER REFERENCES

Journal of the Chemical Society, vol. 112, I, pages 219-220.

Beilstein, vol. 24, pages 111 and 112 (1936).

Berichte, vol. 13, pages 681 and 682 (1880).